

# United States Patent [19]

Wilson

[11] Patent Number: 4,529,405

[45] Date of Patent: Jul. 16, 1985

[54] WATERLESS DYE COMPOSITION AND  
METHOD OF USE THEREOF FOR  
COLORING THERMOPLASTIC MATERIALS

[75] Inventor: Robert B. Wilson, Greenville, S.C.

[73] Assignee: Crucible Chemical Company,  
Greenville, S.C.

[21] Appl. No.: 584,143

[22] Filed: Feb. 27, 1984

[51] Int. Cl.<sup>3</sup> ..... D06P 1/46; D06P 3/00;  
D06P 5/00; D06P 3/52

[52] U.S. Cl. ..... 8/583; 8/506;  
8/508; 8/510; 8/512; 8/513; 8/515; 8/516

[58] Field of Search ..... 8/506, 508, 510, 512,  
8/513, 515, 516, 583

[56] References Cited

U.S. PATENT DOCUMENTS

3,950,419 4/1976 Baumann et al. ..... 8/583  
4,293,305 10/1981 Wilson ..... 8/115.6  
4,394,126 7/1983 Wilson ..... 8/115.6

Primary Examiner—Paul Lieberman

Assistant Examiner—John F. McNally

Attorney, Agent, or Firm—Bailey & Hardaway

[57] ABSTRACT

A waterless dye composition for apparel and other thermoplastic articles comprises a bisterephthalate diester of an alkylphenoxy polyethoxyethanol and an organic colorant. Aromatic polyesters of the formula  $C_6H_2-(COOR_1)_z$ , wherein z is 3, 4, 5, or 6; z' or 6 - z

and R<sub>1</sub> is higher alkyl and/or cycloaliphatic diesters of the formula



wherein R is substituted or unsubstituted straight or branched chain alkyl of 4-20 carbon atoms, polyoxyalkylene of the formula  $HO(C_xH_yO)_nC_xH_y$ —or phosphated polyoxyalkylene of the formula



or a salt thereof, wherein  $(C_xH_{2x}O)_n$  is  $(CH_2CH_2O)_n$ ,  $(C_3H_6O)_n$  or  $(CH_2CH_2O)_p-(C_3H_6O)_q$ , n is 2-22, and the sum of p+q is n can be admixed with the terephthalate composition.

A process for coloring apparel or other articles, fabricated from polyester, polyamide, polyurethane, acrylic, halogenated polyolefin or epoxy plastic, comprises exposing an article to the foregoing compositions, maintained at a temperature between 100° C. and the temperature at which the plastic is degraded, for a time adequate to achieve the desired degree of coloration.

25 Claims, No Drawings.

**WATERLESS DYE COMPOSITION AND METHOD  
OF USE THEREOF FOR COLORING  
THERMOPLASTIC MATERIALS**

**DESCRIPTION**

**1. Technical Field**

This invention relates to waterless compositions, particularly adapted for immersion coloring of plastic articles, whether intended for apparel or general utility applications.

**2. Background Art**

A continuous process for waterless dyeing of textile and plastic materials has been proposed by Hermes in U.S. Pat. Nos. 4,047,889 and 4,055,971. The vehicle disclosed is a high boiling glycol or glycol ether.

The use of alkyl terephthalates, particularly methyl,

$C_6H_z(COOR_1)_z$ , wherein z is 3, 4, 5 or 6; z' is 6-z;  $R_1$  is substituted or unsubstituted higher alkyl or an alkylphenol ether of an alkoxyalkanol and/or a diester of a hydrogenated Diels-Alder adduct of linoleic and acrylic acids. The dye bath for the coloring of thermoplastic articles will contain sufficient amounts of an organic colorant to permit coloring of the thermoplastic articles being dyed.

In another aspect, this invention relates to a process 10 for waterless coloring of thermoplastic articles, fabricated from a plastic composition, comprising exposing an article to the foregoing compositions, maintained at a temperature between 100° C. and the temperature at which the plastic degrades, for a time adequate to 15 achieve the desired degree of coloration.

A bisterephthalate ester of an alkylphenoxypropoxyethanol is a compound of the formula



isopropyl or butyl terephthalates, for dyeing of polyester, polyacrylic or modified cellulosic fibers or fabrics 25 has been proposed by Hallada et al. (U.S. Pat. No. 3,833,613), Landerl (U.S. Pat. No. 2,934,397); Salven et al. (U.S. Pat. No. 2,982,597), Harnett et al. (U.S. Pat. No. 3,667,899) and Forschirm (U.S. Pat. No. 3,973,907). Dellian (U.S. Pat. No. 4,032,291) has proposed the use 30 of phenyl/benzyl phthalates in a similar context.

The use of ethoxylated materials for coloring of objects has been disclosed by Lenz et al. (U.S. Pat. No. 3,362,779) and Kressner et al. (U.S. Pat. No. 4,332,587).

Hinton, Jr. et al., in U.S. Pat. No. 3,824,125, have 35 proposed the use of higher trialkyl trimellitates in laundry compositions to improve soil release properties of synthetic fibers, such as polyesters.

Compositions containing esterified derivatives of a 40 hydrogenated Diels-Alder adduct of linoleic acid and acrylic acid, intended for use in various textile-treating compositions, have been disclosed by Wilson, in U.S. Pat. Nos. 4,293,305 and 4,394,126, incorporated herein by reference.

Although a variety of solvent systems have been 45 suggested for dyeing of articles in waterless systems, none presently available provides rapid, failure-free dyeings, which are done without producing obnoxious effluents or otherwise being unacceptable from a commercial viewpoint.

It is an object of this invention to provide a composition for waterless immersion coloring of plastic articles, produced by the apparel and other industries. Such articles include, but are not limited to buttons, zippers, garments, carpeting, ribbons, draperies, shoe strings, 55 sewing thread, lace, socks, plastic tubing and pipe, plastic coated wire, ropes, polyester and polyamide films, toys, and housings for pencils, pens, kitchen utensils and telephones.

It is a further object of this invention to provide a 60 method for rapid waterless coloring of such articles.

**DISCLOSURE OF THE INVENTION**

In one aspect, this invention relates to a vehicle for waterless dip dyeing of thermoplastic articles, comprising a bisterephthalate ester of an alkylphenoxypropoxyethanol and an organic colorant. The composition can also contain an aromatic polyester of the formula

25 wherein alk is straight or branched chain alkyl of 4-15 carbon atoms and k is 3-20.

It will be understood that alk- $C_6H_5OH$  includes products known as octylphenol, nonylphenol and dodecylphenol, which are alkylation products of propylene or butylene oligomers. These products are, in fact, mixtures of compounds. Nonylphenol, for example, is a technical grade mixture of monoalkylphenols, predominantly para-substituted, in which the side chains are isomeric branchedchain alkyl. Octylphenol may be predominantly 1,1,3,3-tetramethylbutylphenol.

The number of oxyethylene units, designated by "k," also corresponds to a mixture. The product known as nonoxynol is a nonylphenol ether containing, on the average, 15 1,2-oxyethanediyl units (k is 14). The product known as octoxynol is a mixture of polyoxyethylated octylphenol, containing 5-15 oxyethylene units, so that k is 9.

In the bisterephthalate esters, employed as a dye vehicle, it is preferred that the alkylphenol be selected from octylphenol or nonylphenol and that the degree of ethoxylation be 4-6, that is, k is 3-5.

The terephthalate esters are made by reaction between an excess of polyoxyethylated alkylphenol and terephthalic acid or a lower terephthalate ester, e.g., 50 dimethyl terephthalate. Normally, the reaction is carried out under conditions in which water or a lower boiling alcohol is removed from the reaction site by distillation.

"Aromatic polyester," as used in the specification and claims, means an ester formed by reaction between a polybasic aromatic acid of the benzene series and a higher alkanol, so as to accomplish complete esterification of all carboxyl functions therein. "Higher alkanol" means a substituted or unsubstituted alkanol of at least six carbon atoms, for example, hexanol, octanol, 2-ethylhexanol, isodecanol, decanol, hexadecanol, octadecanol, docosanol, oleyl alcohol, linoleyl alcohol or the like.

Also included among "higher alkanols" for the purposes of this invention are alkylphenol ethers of alkoxyalkanols, having the formula



wherein a is 1-12; b is 1-24 and x is 2 or 3, optionally including blocks of ethyleneoxy and propyleneoxy units.

The esters can be made by reaction between, for example, trimellitic acid, and the selected alkanol, conveniently in a fashion so as to remove or entrain by-product water. Alternatively, the aromatic polyesters can be prepared by transesterification between a lower ester, e.g. trimethyl trimellitate and the higher alkanol. In such a reaction, the lower boiling alcohol will normally be removed from the reaction site by distillation.

Contemplated among aromatic polyesters are esters of benzene tetra-, penta- and hexacarboxylic acids, wherein R is as above. Accordingly, esters of phthalic, mellophanic, pyromellitic, trimesic, trimellitic and hemimellitic acids are included, as well as esters of benzenepentacarboxylic acid and mellitic acid.

Although triesters of any of the benzenetricarboxylic acids can be used, it is preferred to use triesters of 1,2,4-benzenetricarboxylic acid, also known as trimellitic acid. Preferred esters are tris(2-ethylhexyl)trimellitate, trisisodecyl trimellitate, trisooctyl trimellitate, tridecyl trimellitate, and trihexadecyl trimellitate. It will be understood that mixed esters, such as hexyl, octyl, decyl trimellitate can also be used. Most preferred is tris(2-ethylhexyl)trimellitate (CAS No. 3319-31-1), also known as trioctyl trimellitate, which can be purchased from Eastman Chemical Products, Inc., Kingsport, Tenn., as Kodaflex® TOTM.

Compositions containing an aromatic polyester as an optional ingredient will preferably contain at least 5% by weight of these materials. The maximum preferred amount of aromatic polyester is about 95% by weight. When binary compositions are contemplated, the amounts of bisterephthalate and aromatic polyester are preferably about equal. Therefore, compositions of 40:60 to 60:40 parts by weight are preferred.

The compositions can also contain a cycloaliphatic diester of the formula



wherein R is substituted or unsubstituted straight or branched chain alkyl of 4-20 carbon atoms, polyoxalkylene of the formula  $\text{HO}(\text{C}_x\text{H}_y\text{O})_n\text{C}_x\text{H}_y-$  or phosphated polyoxalkylene of the formula



or a salt thereof, wherein  $(\text{C}_x\text{H}_y\text{O})_n$  is  $(\text{CH}_2\text{CH}_2\text{O})_n$ ,  $(\text{C}_3\text{H}_6\text{O})_n$  or  $(\text{CH}_2\text{CH}_2\text{O})_p-(\text{C}_3\text{H}_6\text{O})_q$ , n is 2-22 and the sum of p+q is n. Other cycloaliphatic diester compounds which can be used are those wherein R is Ar-COO(CH<sub>2</sub>CH<sub>2</sub>O)<sub>n</sub>CH<sub>2</sub>CH<sub>2</sub>-, ArCOO(C<sub>3</sub>H<sub>6</sub>O)<sub>n</sub>C<sub>3</sub>H<sub>6</sub>-, ArCOO(C<sub>2</sub>H<sub>4</sub>O)<sub>p</sub>(C<sub>3</sub>H<sub>6</sub>O)<sub>q</sub>C<sub>3</sub>H<sub>6</sub>-, or Ar-COO(C<sub>3</sub>H<sub>6</sub>O)<sub>p</sub>-(C<sub>2</sub>H<sub>4</sub>O)<sub>q</sub>C<sub>2</sub>H<sub>4</sub>-, wherein n, p and q are as above and Ar is substituted or unsubstituted mono- or bicyclic aryl of up to 15 carbon atoms. It is preferred that compositions of this invention contain at least 5% by weight of one or more of these cycloaliphatic diesters.

Binary compositions containing bisterephthalate and cycloaliphatic diesters will preferably contain at least 5% by weight of one or more of these materials. The maximum preferred amount is about 95% by weight of the cycloaliphatic diester. It is most preferred that the amounts of bisterephthalate and cycloaliphatic diester are about equal, so that compositions of 40:60 to 60:40 parts by weight are preferred.

Ternary vehicles for waterless dip dyeing will contain at least 5% by weight of each of a bisterephthalate ester, an aromatic polyester and a cycloaliphatic diester. A most preferred compositional range is that comprising 60-80% by weight of aromatic polyester and 10-20% by weight of each of the other esters.

The dibasic cycloaliphatic acid employed in making the compositions of this invention is a Diels-Alder adduct of acrylic acid and linoleic acid and can be prepared as described by Ward in U.S. Pat. No. 3,753,968. The diacid has the formula



and therefore is a mixture of (5 and 6)-carboxy-4-hexyl-2-cyclohexane-1-octanoic acids. The diacid is available commercially from Westvaco, designated as "Diacid 1550".

Preparation of adducts from conjugated octadecadienoic acid and unsaturated acids and/or their hydrogenation has also been described by Teeter et al, *J. Org. Chem.*, vol. 22 (1957) at 512-514, Ward in U.S. Pat. No. 3,899,476 and Ward et al in U.S. Pat. No. 3,981,682.

The preparation of esters from the C<sub>21</sub> diacid adduct was reported by Ward et al, *J. Amer. Oil Chemists' Soc.*, vol. 57 (1957) at 219-224. Ethoxylated esters containing 4-119 ethylene oxide units are said to be effective lime soap dispersants. The alkyl esters are reported as being useful in lubricant applications, including use as textile lubricants and plasticizers for PVC.

The diacid can be esterified with alcohols using, for example, acidic catalysts such as p-toluenesulfonic acid, methanesulfonic acid or sulfuric acid. During the esterification, the reaction mixture is preferably also treated with a decolorizing agent, e.g., carbon or clay.

The diacid is reduced following esterification to a saturated compound. A nickel catalyst such as Raney Nickel, nickel on kieselguhr or nickel on alumina can be used. The required amount varies up to 5-10% by weight of the ester.

Hydrogenation is carried out after esterification to prevent nickel from complexing with the free acid. Other catalysts, e.g., platinum or rhodium, avoid this problem, but are prohibitive in cost. The catalyst can be removed by filtration through a plate and frame filter press. The product is the resulting filtrate.

Polyoxalkylene diesters are prepared by reaction of the diacid, in the presence of an alkaline catalyst, with ethylene or propylene oxide. Reaction will occur at both acid sites. Addition of ethylene oxide is allowed to continue until the product becomes at least dispersible or, preferably, soluble in water. This will correspond to addition of a total of 5-25 ethylene oxide units. The product obtained using ethylene oxide has a structure before hydrogenation represented by the formula:



The phosphorylated product is readily obtained by reaction with phosphorus pentoxide. The saturated diester can be obtained by nickel-catalyzed hydrogenation.

In the case of the phosphorylated derivative, hydrogenation should precede phosphorylation. The phosphorylated derivatives can be converted to salts thereof by reaction with a metal hydroxide. Sodium and potassium salts are preferred.

Compounds in which R is  $\text{ArCOO}(\text{CH}_2\text{CH}_2\text{O})_n\text{CH}_2\text{CH}_2-$ , etc. are obtained by treating polyoxalkylene intermediates with an aromatic acid, e.g., 10 benzoic, toluic or mellitic acid, usually with an acidic catalyst. Hydrogenation of the double bond in the cycloaliphatic ring can be done before or after esterification with the aromatic acid.

Representative of substituted alkyl R which may be 15 used in the products of this invention are butoxybutyl, 10-hydroxystearyl, 10-hydroxydecyl, 10-halostearyl,  $\omega$ -alkanoyloxyalkyl or the like.

Preferred cycloaliphatic diesters for use in accordance with the principles of the invention are those 20 wherein:

- (a) R is straight or branched chain alkyl of 4-20 carbon atoms,
- (b) R is 2-ethylhexyl, lauryl or stearyl,
- (c) R is  $\text{HO}(\text{CH}_2\text{CH}_2\text{O})_n\text{CH}_2\text{CH}_2-$ ,
- (d) R is  $\text{HO}(\text{C}_3\text{H}_6\text{O})_n\text{C}_3\text{H}_6-$ ,
- (e) R is  $\text{HO}(\text{C}_2\text{H}_4\text{O})_p(\text{C}_3\text{H}_6\text{O})_q\text{C}_3\text{H}_6-$ ,
- (f) R is  $(\text{HO})_2\text{P}=\text{O}(\text{OCH}_2\text{CH}_2)_n\text{OCH}_2\text{CH}_2-$  or a salt thereof,
- (g) R is  $\text{C}_6\text{H}_5\text{CO}(\text{OC}_2\text{H}_4)_n\text{OC}_2\text{H}_4-$ ,
- (h) R is  $\text{CH}_3\text{C}_6\text{H}_4\text{CO}(\text{OC}_2\text{H}_4)_n\text{OC}_2\text{H}_4-$ ,
- (i) R is  $\text{C}_6\text{H}_5\text{CO}(\text{OC}_3\text{H}_6)_n\text{OC}_3\text{H}_6-$ , and
- (j) R is  $\text{CH}_3\text{C}_6\text{H}_4\text{CO}(\text{OC}_3\text{H}_6)_n\text{OC}_3\text{H}_6-$ .

The types of plastic materials which can be colored using the compositions and method of this invention include, but are not limited to, polyesters, polyamides, polyurethanes, acrylics, halogenated polyolefins and epoxy plastics. However, textile- and apparel-related articles are commonly made from polyesters, polyamides, polyurethanes and acrylics, which substrates are preferred for the practice of this invention. Pipe and tubing are commonly made from chlorinated polyethylene (CPE) or post-chlorinated PVC (PCPVC).

Polyester articles include those made from poly(alkylene terephthalates), such as poly(ethylene terephthalate), or polyesters made from cyclohexanedimethanol. Typical of polyester articles are presewn garments, including slacks, jeans, dresses shirts, scarves and the like. Also included within the scope of polyester articles are buttons, draperies, laces, seatbelts, ribbons, zippers and other notions, as well as chips of polyester resins, polyester coatings on wire or metal, polyester articles (including those made from styreneated polyesters), polyester film, toys, components of automobiles and airplanes and housings for pencils, pens or household articles.

Polyamides particularly contemplated as substrates in the practice of this invention include those known as nylons 6, 6,6 or 6,10. Articles which can be colored in

accordance with the invention include the same types of articles as for polyesters, as well as lingerie and hosiery. It is common, for example, to employ polyamide teeth in zipper constructions. Polyamides are often used for carpeting and ropes.

Acrylic plastics, contemplated within the scope of this invention include straight acrylics, such as polyacrylonitrile, and modacrylics. The latter are copolymers of acrylonitrile or methacrylonitrile, generally with vinyl chloride or vinylidene chloride. Articles made from acrylics include clothing, carpeting and notions.

Also included among acrylics are high impact resins, whether comprising blends or graft copolymers. These are commonly identified as ABS resins. Articles made therefrom include chips, coatings for wire and metal, telephone housings, toys, impact-resistant moldings for automobiles and airplanes, and housings for pencils, pens and kitchen utensils.

Polyurethanes include a myriad of compositions, made by reaction, for example, between glycols and organic di- or polyisocyanates. Among the glycols, used to make polyurethanes, are simple glycols, such as the alkylene glycols, and polymeric glycols, including polyether and polyester glycols. Articles containing polyurethane, include rain wear, artificial leather, toys, and moldings and extrusions for automobiles and airplanes. Any of these articles can be colored by the teachings of the instant invention.

In some instances, the foregoing types of plastics can be blended with natural or synthetic cellulosic materials and colored according to this invention.

"Organic colorant," as used in the specification and 35 claims, includes both dyes and pigments of any structure. Normally, the dyes or pigments which are employed need not be soluble in water. Therefore, such dyes and pigments will not usually contain water-solubilizing functions, such as a plurality of sulfonic acid groups. The dyes/pigments used in the practice of 40 this invention generally will be chosen from among water-insoluble dyes, which may also be known as disperse dyes. Included within this class of dyes, which can be used on fibers such as cellulose acetate, polyamides or polyesters, from any kind of dyeing medium are 45 colors of azo, azomethine, nitroarene and anthraquinone structures. It will be understood that the dyes useful in the practice of the present invention are not limited to these classes of compounds.

The dyes or pigments used in the practice of this 50 invention may be identified by their chemical names, for example:

3-nitro-N<sup>4</sup>-phenylsulfanilanilide, a yellow dye; p-[p-(phenylazo)phenylazo]phenol, a red-yellow dye; ethyl 4-hydroxy-1-anthraquinonecarbamate (an orange dye); 1-amino-4-hydroxyanthraquinone, a red dye; 1-amino-2-bromo-4-hydroxyanthraquinone, a red-blue dye or 4,5-diaminochrysazin, a blue dye.

The dyes alternatively may be identified in accordance with standard chemical handbooks, such as "The Color Index," third edition, The Society of Dyes and Colors and the American Association of Textile Chemists and Colorists (1971). This sort of handbook correlates dye structure with trade names. Typical of colorants identified in accordance with this handbook, which can be used in the practice of this invention, are Solvent 55 Orange 20; Acid Blue 83 (C.I. 42660), Acid Blue 59

(C.I. 50315), Direct Blue 86 (C.I. 74180); Direct Red 81 (C.I. 28160) and Acid Yellow 36 (C.I. 13065).

Cationic dyestuffs can also be used in the practice of this invention, for example Rhodamine 6G, Rhodamine B, Rhoduline Blue 6G and Methylene Blue BB.

Similarly, metallized azo dyestuffs can be employed in the practice of this invention. Representative metallized azo dyes which can be employed are Co, Ni, Cu or Cr complexes of coupling products of 2-amino-4-nitrophenol and resorcinol; 2-amino-4-chloro-5-nitrophenol and acetoacetanilide; dianisidine and 3-hydroxy-2-naphthaniilide; 2-amino-4-chloro-5-nitrophenol and 2-aminonaphthalene or the like.

It will further be understood that other textile-treating agents, such as optical brighteners, e.g. styrylnaphthoxazole compounds, can be applied, along with dyes or pigments.

The dyes/pigments can be used in any form, that is, as presscake or as dried pressed dye. The addition of dispersing agents is optional. Alternatively, the dyes or pigments can be added to the dye bath in a solvent/dispersing medium compatible with the dye bath. It is convenient and preferred, in the practice of this invention, to use solid disperse dyes free of additives.

It has been found that waterless dye baths containing at least 5% by weight of an aromatic polyester can be decolorized using activated carbon, whereas baths of prior art compositions, containing no aromatic polyester are not readily decolorized in this fashion.

Addition of triphenyl phosphite to the dye baths has been found to reduce discoloration of the dye bath. Accordingly, compositions containing 0.1-2.0% by weight of triphenyl phosphite are preferred.

Optional dyeing assistant agents, used in the compositions of this invention, include alkoxylated alkylphenols and their esters, alkoxylated castor oil compounds, alkoxylated hydrogenated castor oil compounds, alkoxylated primary alkanols, salts of phosphated alkoxylated primary alkanols and mixtures thereof. These optional dyeing assistant agents will preferably be utilized as lubricant, spin finishing or dyeing bath additives, for aqueous dye baths, in accordance with Wilson, U.S. Pat. Nos. 4,293,305 and 4,394,126.

The amount of optional dyeing assistant agent, employed in the compositions of this invention, is at least about 0.5% by weight of the composition.

Preferred compositions for these purposes can also contain 60-80% by weight of one or more optional dyeing assistant agents.

Preferred optional dyeing assistant agents are alkoxylated alkylphenols and their esters. These are compounds of the formula



wherein a is 1-12; b is 1-24; R'' is H, aroyl of mono- or bicyclic aromatic acids of up to 15 carbon atoms or substituted or unsubstituted alkanoyl of 8-30 carbon atoms. Accordingly, exemplary dyeing assistant agents include ethoxylated and propoxylated alkyl phenols and corresponding esters, such as the laurate, myristate, palmitate, coconate, oleate, stearate, isostearate, benzoate and toluate esters. Preferred alkylphenols are nonylphenol, octylphenol, and dodecylphenol.

It will be understood that the alkylphenols and the acids used to esterify the alkoxylated alkylphenols can include mixtures.

Most preferably, the alkoxylated alkylphenols will be ethoxylated derivatives, having 5-10 ethylene oxide units.

Preferred optional dyeing assistant agents will be those wherein:

- (a) R'' is alkanoyl of 12-18 carbon atoms, including mixtures thereof;
- (b) R'' is n-C<sub>17</sub>H<sub>33</sub>CO;
- (c) R'' is n-C<sub>17</sub>H<sub>35</sub>CO;
- (d) R'' is iso-C<sub>17</sub>H<sub>35</sub>CO;
- (e) R'' is benzoyl;
- (f) R'' is n-C<sub>11</sub>H<sub>23</sub>CO;
- (g) R'' is H;
- (h) a is 5-10, including each of (a)-(g);
- (i) b is 6-15, including each of (a)-(h);
- (j) b is 8-11, including mixtures thereof and including each of (a)-(h);
- (k) a is 9, b is 8-10 and R'' is n-C<sub>11</sub>H<sub>23</sub>CO;
- (l) a is 9, b is 6-10 and R'' is H and
- (m) x is 2, including each of (a)-(l).

Alkoxylated castor oil used as optional additives in the compositions of this invention will contain 15-100 oxyalkylene units, preferably 40-85 oxyethylene units. The hydrogenated cator oil derivatives will contain 5-200 oxyalkylene units, preferably 20-30 oxyethylene units. These types of materials can be purchased from ICI America and Whitestone Chemical Co.

It has been found, in accordance with this invention that articles can be dyed or colored very rapidly and very homogeneously. Normally, immersion in the dye bath for as little as 30 seconds at 160° C. will give significant coloration. However, for even faster results, the dyeings can be done at 180°-200° C. or higher. Employing the compositions of this invention at 200° C. or more does not result in smoking or pollution of the processing plant, which is a problem when ethylene glycol or diethylene glycol are the dyeing solvents. In practice, it is feasible to use a temperature, up to that at which the plastic being dyed, will degrade. However, temperatures between 120°-235° C., most preferably 140°-235° C., will be preferred.

Although it is preferred to dye the articles being treated by immersion in a bath of the dye composition, the dyes can also be applied by spraying. Then, the sprayed articles should be heated in a bath to at least 140° C. to complete uptake of the dye into the article.

Whether the article is dyed by immersion or otherwise, the dyed article is normally cleaned with a solvent to remove excess dye. Preferably, the solvents used for cleaning are chlorinated or fluorinated hydrocarbons. However, highly chlorinated solvents, such as perchloroethylene and trichloroethylene are preferred for cleaning by immersion in a liquid bath. Fluorochlorocarbons, such as dichlorodifluoromethane, chlorotrifluoromethane, which are gases at ambient temperatures or slightly above, can be used for vapor-phase cleaning of the dyed articles. Normally, means will be used to recover and recycle the cleaning solvent, rather than discharging it to the atmosphere.

A further advantage of the process of the invention is that it is essentially self-contained and effluent free, that is, little or no material is lost or discharged to the atmosphere.

In the apparatus of this invention, the major components include a dip tank, a dye recovery unit, a solvent cleaning tank, a solvent recovery still and a drier. The dip tank will be provided with heating means and stirring means, so as to permit circulation of the dyeing

solution within the dip tank and to a dye recovery unit external thereto.

The dye recovery unit normally includes filtration means for removal of solid debris from used dye solutions and distilling and condensing means for recovery of the solvent. The purified dye solution can be recycled to the dip tank, with addition of dye or other additives to provide the desired composition in the dip tank, or can be stored for later use.

It is preferred, in coloring many types of textile-related articles, including jeans, shorts, lingerie, carpeting, hosiery, zippers and lace, as exemplary, to provide squeeze roller means, essentially functioning as wringers, to remove excess dye solution from treated articles. The dye solution removed at this point can be cycled to the external recovery unit or can be returned directly to the dip tank.

When the dye bath contains at least 5% by weight of aromatic polyester and is free of other optional dyeing assistant agents, it is preferred to recover clean dye vehicle by treatment with activated carbon. This treatment permits reuse of the dyeing vehicle with a plurality of different organic colorants and avoids the need for recovering the dyeing vehicle by distillation.

Articles leaving the squeeze roll station are passed into the solvent cleaning tank to complete removal of any excess or unadherent dye matter. It is preferred to use a plurality of solvent cleaning tanks. It is also preferred to circulate solvent from the tank through an external solvent recovery unit, provided with filters to remove solid materials and distilling and condensing means for purifying solvent, and to return purified solvent to the system. Dye recovered on the filter or as residue from the distillation can be returned to the system for recycle. When a plurality of solvent cleaning tanks are employed, it is preferred to flow solvent countercurrently to the direction in which the articles being treated, are moved.

The final component of the apparatus is the drying means, such as a hot air drier, from which articles leaving the system can be inspected and packaged. Solvent vapors from the hot air drier can be condensed and returned to the system.

#### BEST MODE FOR CARRYING OUT THE INVENTION

In a most preferred aspect, the compositions of this invention will contain 40-60% by weight of either aromatic polyester or cycloaliphatic diester and 0.05-2.0% by weight of triphenyl phosphite. In compositions containing an aromatic polyester, a trialkyl trimellitate in which alkyl is of 6-20 carbon atoms is preferred. In compositions containing a cycloaliphatic diester, one is preferred wherein R is of 6-20 carbon atoms. Preferred ternary compositions will contain 60-80% by weight of aromatic polyester, 10-20% by weight of each of the other esters and 0.05-2.0% by weight of triphenyl phosphite. Bisterephthalate esters in which k is 3-5, are preferred. The preferred organic colorant is a disperse dye.

A most preferred process in accordance with this invention is one wherein the article being treated is exposed to one of the foregoing compositions, maintained at a temperature of 140°-235° C. for a time adequate to achieve the desired degree of coloration.

Without further elaboration, it is believed that one skilled in the art can, using the preceding description, utilize the present invention to the fullest extent. The

following specific embodiments are, therefore, to be construed as merely illustrative and not limitative of the remainder of the disclosure in any way whatsoever. In the following examples, the temperatures are set forth uncorrected in degrees Celsius. Unless otherwise indicated, all parts and percentages are by weight.

#### EXAMPLE 1

##### Preparation of Polyoxyethylene Nonylphenyl Laurate

To a three-necked flask fitted out with stirrer, condenser, receiver, thermometer, nitrogen purge and heating mantle were charged 750 g (1.1 moles) of polyoxyethylated nonylphenol (9.5 moles of oxyethylene, NP 9.5), 208 g (1 mole) of lauric acid and 2.4 g of p-toluenesulfonic acid. Air was purged from the flask with nitrogen and the mixture was heated to 160°-170° C. Water was removed continuously. The reaction was allowed to continue until an acid value below 10 mg/KOH was obtained for a sample of product. The product was cooled and filtered.

Other polyoxyethylene compounds are made in a similar fashion from:

- (1) NP 9.5 and coconut fatty acid, 1:1 molar ratio
- (2) NP 9.5 and oleic acid, 1:1 molar ratio
- (3) NP 9.5 and stearic acid, 1:1 molar ratio
- (4) NP 9.5 and benzoic acid, 1:1 molar ratio.

#### EXAMPLE 2

##### Preparation of Cycloaliphatic Diester (R is 2-ethylhexyl)

To a three-necked flask fitted with stirrer, thermometer, nitrogen purge, condenser, side-arm receiver and heating mantle were charged 352 g (1 mole) of Diacid 1550, 273 g (2.1 moles) of 2-ethylhexanol, 1.5 g of p-toluenesulfonic acid and 2 g of decolorizing carbon. Air was purged from the flask with nitrogen and the reaction mixture was stirred and heated to 160°-170° C. for 4-6 hours. Water formed during the reaction was collected in the side-arm receiver. The reaction was continued until the acid value was below 5 mg KOH/g. The catalyst and carbon were removed by filtration. The ester product and 25 grams of nickel on kieselguhr were charged to a stirred, heated pressure vessel. The mixture was heated to 160°-170° C. and pressurized to 400 psig with hydrogen. A sample was removed after 6-8 hours for determination of the iodine value. The reaction was continued until the iodine value was below 0.5 g of iodine/100 g of sample.

The product was cooled to 50° C. and the catalyst was removed by filtration.

Esters are prepared similarly from:

- (1) Diacid 1550 and decyl alcohol, 1:2 molar ratio
- (2) Diacid 1550 and tridecyl alcohol, 1:2 molar ratio
- (3) Diacid 1550 and Neodol 25 (a mixture of 12-15 carbon alcohols), 1:2 molar ratio.

#### EXAMPLE 3

##### A. Preparation of Polyoxyethylene Unsaturated Cycloaliphatic Diester, R is $\text{HO}(\text{CH}_2\text{CH}_2\text{O})_n\text{CH}_2\text{CH}_2-$

To a stirred autoclave fitted with heating and cooling coils was charged 352 g (1 mole) of Diacid 1550. Catalyst (1.0 g of potassium hydroxide) was charged to the reactor. The temperature was raised to 110° C. and the reactor was vacuum stripped for 30-60 minutes to remove any residual water from previous washing of the

reactor or from one or more of the charged reactants or catalyst. The reactor was purged with nitrogen to remove air, evacuated again and purged again with nitrogen. The contents of the reactor were stirred and heated to 140° C. and 100 g (2.3 moles) of ethylene oxide was added to the reactor. The pressure inside the reactor immediately built up to 30–50 psig. After 30–60 minutes' induction time, an exothermic polymerization reaction (to 150°–160° C.) began. The reaction was accompanied by a pressure drop to zero (0 psig) as the ethylene oxide was consumed. Ethylene oxide was added to the reactor to a total of 660 g (15 moles). The temperature was maintained at 150°–160° C. by cooling. Addition of ethylene oxide was stopped and the reaction was allowed to continue for 30 minutes more. The reactor was cooled to 90°–100° C. and purged twice with nitrogen.

A sample of the product had a hydroxyl value of 110 mg of KOH/g (15 moles of ethylene oxide added to the diacid.) The diester was acidified with acetic acid to neutralize the potassium hydroxide catalyst and treated with 3 g of hydrogen peroxide to bleach and lighten the color of the product. The reactor was cooled to 30° C. prior to removing the product, which was filtered through filter paper, using a porcelain filter.

#### B. Reduction to the Polyoxyethylene Diester

The product of Example 3A and 25 g of nickel on kieselguhr were charged to a stirred, heated pressure vessel. The mixture was heated to 160°–170° C. and pressurized with hydrogen to 400 psig. After 6–8 hours, samples were removed at intervals for determination of the iodine value. The reaction was continued until the iodine value was less than 0.5 g/100 g of sample.

#### EXAMPLE 4

##### Preparation of Phosphated Polyoxyethylene Diester (R is $(\text{HO})_2\text{P}(=\text{O})(\text{OCH}_2\text{CH}_2)_n-\text{OCH}_2\text{CH}_2-$ )

Polyoxyethylated (15 moles of ethylene oxide) diacid, obtained as in Example 3B was heated to 50°–60° C., stirred and purged thoroughly with nitrogen to remove air. To about 1015 g (1 mole) of this material was added 24 g (0.17 mole) of phosphorus pentoxide. An exothermic reaction began immediately, with an exotherm to 85°–95° C. The reaction mixture was maintained at this temperature by cooling and an additional 24 g (0.17 mole) of phosphorus pentoxide was added. The reaction was continued for three hours after all of the phosphorus pentoxide was added. The reactor was cooled to 50° C. prior to removal of a sample. The acid value of the product was 32 mg KOH/g, indicating that the reaction was complete. The batch was bleached at 85°–95° C. with 5 g of hydrogen peroxide, cooled to 30° C. and filtered.

#### EXAMPLE 5

##### Aroylpolyoxyethylene Cycloaliphatic Diester

An aroylpolyoxyethylene cycloaliphatic diester was synthesized in a two-liter autoclave fitted with nitrogen purge, condenser and receiver for the removal of by-product water. Charge weights were:

510.0 g.: Diacid 1550

2.0 g.: flake caustic

636.0 g.: ethylene oxide

After purging the system with nitrogen, Diacid 1550 and caustic were heated to 130° C. Ethylene oxide was added over a four-hour period, during which the temperature was kept at 150°–165° C. The resulting ethoxylated product was cooled to 90° C. for removal of a

sample. The hydroxyl value was 139. To this intermediate was added:

3.5 g.: acetic acid (glacial)

7.5 g.: methanesulfonic acid (70%)

340.0 g.: benzoic acid

After purging with nitrogen, the temperature of the mixture was raised to and held at 165°–170° C. until the acid value was less than 5 mg KOH per gram. The theoretical amount of water was removed during the reaction and collected in the receiver. The sample was cooled and filtered.

The filtered product was hydrogenated in a two-liter autoclave:

1000.0 g: ethoxylated product, above

50.0 g: Raney nickel

QS: hydrogen

The reduction was run at 100°–125° C. and 200–250 psig until hydrogen consumption ceased. The product was cooled and filtered.

#### EXAMPLE 6

Ethoxylated castor and hydrogenated castor oils were prepared as in Example 3. Ethylene oxide adds to the hydroxyl group of castor oil.

#### EXAMPLE 7

Bisterephthalate ester is prepared from polyoxyethylated nonylphenol (about 5 oxyethylene units) by heating with dimethyl terephthalate, until distillation of methanol ceases.

#### EXAMPLE 8

35 (a) A waterless dyeing composition was prepared from bis(2-ethylhexyl)cycloaliphatic diester of Example 2 and the bisterephthalate ester of Example 7 in 45:55 weight ratio. The dye composition also contained 5 grams/liter of Disperse Blue 60 and 0.2% by weight of triphenyl phosphite.

40 This composition was kept at 185° C. and stirred while a piece of polyester carpet was immersed therein for 30 sec. The carpet section was removed, washed in perchloroethylene and dried. The carpet was homogeneously colored with good dye fixation. There was little or no smoking during the coloring operation.

45 (b) Similar results were obtained by dyeing a polyamide carpet swatch under the same conditions.

#### EXAMPLE 9

50 A vehicle for dip dyeing was made from 45 parts by weight of the bisterephthalate ester of Example 7 and 55 parts by weight of tris(2-ethylhexyl)trimellitate, containing 0.2% by weight of triphenyl phosphite.

To this was added Disperse Blue 56 at a level of 5 g/l. 55 The resulting composition was used to dye a piece of nylon carpet (185° C., 30 sec) as in Example 8. Similar results were obtained.

#### EXAMPLE 10

60 Dye vehicles containing 0.2% by weight of triphenyl phosphite were prepared from:

|                                          | parts by weight |    |    |
|------------------------------------------|-----------------|----|----|
| tris(2-ethylhexyl) trimellitate          | 70              | 70 | 9  |
| bis(2-ethylhexyl) cycloaliphatic diester | 20              | 10 | 50 |
| bisterephthalate of Example 7            | 10              | 20 | 41 |

Samples of nylon and polyester carpet were dyed successfully at 185° C. (30 sec) with the above compositions, containing 5 g/l of Disperse Blue 56.

## EXAMPLE 11

Dye solution, containing 5 grams of Disperse Blue 56 and 0.2% by weight of triphenyl phosphite in the bis-terephthalate ester of Example 7 were used to dip dye carpet samples of both nylon and polyester. The composition gave acceptable dyeing results.

10

## EXAMPLE 12

An apparatus for removal of dye solutions of the invention consisted of three stainless steel columns, each 5 cm in diameter and 50 cm long. Each column was fitted with a circular pad (5 microns), in the center of which was a hole 0.64 cm in diameter. The pad was covered with a disc of stainless steel screen and topped with Whatman no. 1 filter paper.

15

The first column of the series was packed with 100-200 g of activated granular carbon (Calgon Corp.) and was used as a holding tank for heating the dye solution to about 185° C.

Each of the second and third columns was packed with about 500 g of activated carbon. The temperature 20 of the liquid being passed through these columns was about 185° C. and 120° C., respectively.

25

Dye solutions (Disperse Blue 60 at a concentration of 5 g/l) in 80:20 tris(2-ethylhexyl)trimellitate: bis(2-ethylhexyl)cycloaliphatic diester by volume were decolorized in the foregoing series of three columns. About 15.5 liters of dye solution was decolorized by about 500 g of activated granular carbon. At a dye concentration of 5 g/liter, 1 pound of carbon will accordingly decolorize about 30 pounds of dye mixture.

Flow rates were varied from very slow to a rate of 1 gal/minute/square foot of surface area without adversely affecting recovery of the vehicles.

The foregoing apparatus was used for the decolorization of dye solutions, containing 5-10 g/l of about 60 different dye formulations. The process need not be carried out under an inert atmosphere.

40

The preceding examples can be repeated with similar success by substituting the generically or specifically described reactants and/or operating conditions of this invention for those used in the preceding examples.

45

From the foregoing description, one skilled in the art can easily ascertain the essential characteristics of this invention and, without departing from the spirit and scope thereof, can make various changes and modifications of the invention to adapt it to various usages and conditions.

It is claimed:

1. A waterless dip dye composition for apparel or other thermoplastic articles, comprising a bis-terephthalate ester of the formula

55



60

wherein alk is straight or branched chain alkyl of 4-15 carbon atoms and k is 3-20, and an organic colorant.

2. The composition of claim 1, containing at least 5% by weight of at least one material selected from:

65

an aromatic polyester of the formula C<sub>6</sub>H<sub>2</sub>(COOR<sub>1</sub>)<sub>2</sub>, wherein R<sub>1</sub> is substituted or unsubstituted alkyl of

6-22 carbon atoms or the residue of an alkylphenol ether of an alkoxyalkanol; z is 3, 4, 5, or 6; z' is 6-z and

a cycloaliphatic diester of the formula



wherein R is substituted or unsubstituted straight or branched chain alkyl of 4-20 carbon atoms, polyoxyalkylene of the formula R'(OC<sub>x</sub>H<sub>2x</sub>)<sub>n</sub> or phosphated polyoxyalkylene of the formula (HO)<sub>2</sub>P(=O)(OC<sub>x</sub>H<sub>2x</sub>)<sub>n</sub>OC<sub>x</sub>H<sub>2x</sub>- or a salt thereof, wherein (C<sub>x</sub>H<sub>2x</sub>O)<sub>n</sub> is (C<sub>2</sub>H<sub>4</sub>O)<sub>n</sub>-, (C<sub>3</sub>H<sub>6</sub>O)<sub>n</sub>- or (C<sub>2</sub>H<sub>4</sub>O)<sub>p</sub>(C<sub>3</sub>H<sub>6</sub>O)<sub>q</sub>-; R' is H or ArCO; Ar is substituted or unsubstituted mono- or bicyclic aryl of up to 15 carbon atoms; x is 2 or 3; n is 2-22 and the sum of p+q is n.

3. The composition of claim 2, containing at least 5% by weight of the aromatic polyester.

4. The composition of claim 3, containing at least 5% by weight of a trialkyl trimellitate, wherein alkyl is of 6-22 carbon atoms.

5. The composition of claim 2, containing at least 5% by weight of cycloaliphatic diester, wherein R is alkyl of 6-20 carbon atoms.

6. The composition of claim 1, wherein the bis-terephthalate ester is made from polyoxyethylated nonylphenol or octylphenol and k is 3-5.

7. The composition of claim 2, containing at least 5% by weight of an aromatic polyester and 5% by weight of a cycloaliphatic diester.

8. The composition of claim 1, which contains 0.05-2.0% by weight of triphenyl phosphite.

9. The composition of claim 1, wherein the organic colorant is a disperse dye.

10. The composition of claim 1, consisting essentially of 40-60% by weight of bis-terephthalate ester, 40-60% by weight of cycloaliphatic diester, wherein R is alkyl of 6-22 carbon atoms, 0.05-2.0% by weight of triphenyl phosphite and organic colorant.

11. The composition of claim 10, wherein the bis-terephthalate ester is from nonylphenol, k is 3-5 and the cycloaliphatic diester is the bis(2-ethylhexyl)diester.

12. The composition of claim 1, consisting essentially of 40-60% by weight of bis-terephthalate; 40-60% by weight of aromatic polyester, 0.05-2.0% by weight of triphenyl phosphite and organic colorant.

13. The composition of claim 12, wherein the bis-terephthalate ester is from nonylphenol or octylphenol, k is 3-5 and the aromatic polyester is a trialkyl trimellitate.

14. The composition of claim 1, consisting essentially of 60-80% by weight of aromatic polyester, 10-20% by weight of bis-terephthalate ester, 10-20% by weight of cycloaliphatic diester, 0.05-2.0% by weight of triphenyl phosphite and an organic colorant.

15. The composition of claim 14, wherein the aromatic polyester is a trialkyl trimellitate, the cycloaliphatic diester is one wherein R is alkyl of 6-22 carbon atoms, the bis-terephthalate ester is from octylphenol or nonylphenol and k is 3-5.

16. A process for coloring articles, made from plastic, comprising exposing an article being treated to a composition of claim 1, maintained at a temperature from 100° C. to the temperature at which the plastic degrades, for a time adequate to achieve the desired degree of coloration.

17. The process of claim 16, wherein the plastic is polyester, polyamide, polyurethane, acrylic, halogenated polyolefin or epoxy.

18. The process of claim 16, wherein the article is immersed in the coloring composition at a temperature of at least 140° C. for at least 30 seconds.

19. The process of claim 16, wherein the article is sprayed with the coloring composition and heated in a bath or oven to at least 140° C.

20. The process of claim 16, including the further steps of cleaning the colored article with a halogenated solvent and drying the thus-cleaned article.

21. The process of claim 20, wherein the halogenated solvent is perchloroethylene or trichloroethylene and the halogenated solvent is collected and recycled to the process.

22. A process for coloring articles, made from polyester, polyamide, polyurethane, acrylic, halogenated polyolefin or epoxy plastic, comprising exposing an article being treated to a waterless coloring composition of claim 2, maintained at 120°-235° C., for a time adequate to achieve the desired degree of coloration.

23. The process of claim 22, wherein the article is immersed in the coloring composition at a temperature of at least 140° C. for at least 30 seconds.

24. The process of claim 1, including the further steps of drying the colored article, cleaning the article with a halogenated solvent and drying the thus-cleaned article.

25. A process for coloring articles, made from polyester, polyamide, polyurethane, acrylic, halogenated polyolefin or epoxy plastic, comprising exposing an article being treated to a waterless coloring composition of claim 3, maintained at 120°-235° C. for a time adequate to achieve the desired degree of coloration, wherein the coloring composition is treated after use with activated carbon to recover the waterless medium for use with another organic colorant.

\* \* \* \* \*

25

30

35

40

45

50

55

60

65